

# United States Patent Office

3,338,661

Patented Aug. 29, 1967

1

3,338,661

**CELLULOSIC FABRICS RENDERED CREASE RESISTANT AND WATER REPELLENT THROUGH TREATMENT WITH COMPOSITIONS COMPRISING CATALYST-WATER REPELLENT SILICONES AND SULFONE CROSSLINKING AGENTS**

John W. Gilkey, Midland, Mich., assignor to Dow Corning Corporation, Midland, Mich., a corporation of Michigan

No Drawing. Filed Oct. 28, 1964, Ser. No. 407,210  
12 Claims. (Cl. 8—115.6)

This invention relates to a method of producing a fabric which is both crease resistant and water repellent.

The use of various organic resins to make cellulosic fabrics crease resistant has been well established. In general, these resins are of the ultra-aldehyde or melamine-aldehyde type. Whereas these resins give excellent crease resistance they suffer from the disadvantage that the fabrics so treated lose strength on exposure to bleaching powder and subsequent heating. Recently, various sulfones hereinafter described have been advocated for this use. These sulfones have the advantage that they are stable to alkaline bleach. However, it has not heretofore been commercially feasible to simultaneously treat fabrics with these sulfones and with silicone water repellents. Applicant has found unexpectedly that such simultaneous treatment can be obtained by employing the combination set forth below.

It is an object of this invention to produce a novel method of treating cellulosic fabrics which will render them both crease resistant and water repellent. Other advantages will be obvious to those skilled in the art.

This invention relates to a method comprising contacting a cellulosic fabric with an aqueous dispersion of a mixture of

(1) A sulfone selected from the group consisting of divinyl sulfone,  $\text{CH}_2=\text{CHSO}_2\text{CH}_2\text{CH}_2\text{Z}$ ,

$\text{ZCH}_2\text{CH}_2\text{SO}_2\text{CH}_2\text{CH}_2\text{Z}$ ,  $\text{ZCH}_2\text{CH}_2\text{SO}_2\text{XSO}_2\text{CH}_2\text{CH}_2\text{Z}$  and  $\text{CH}_2=\text{CHSO}_2\text{CH}_2\text{CH}_2\text{NR}_n\text{NCH}_2\text{CH}_2\text{SO}_2\text{CH}=\text{CH}_2$  in which:

$\text{Z}$  is of the group consisting of  $-\text{SSO}_3\text{M}$ ,  $-\text{OSO}_3\text{M}$ , quaternary ammonium salt residues attached to the  $\text{CH}_2\text{CH}_2$  group through carbon-nitrogen bonds, and  $\text{OR}'$  groups in which

$\text{M}$  is an anion,

$\text{R}'$  is of the group hydrogen, lower aliphatic hydrocarbon radicals and acyl radicals derived from lower aliphatic carboxylic acids,

$\text{R}$  is a divalent hydrocarbon radical, any valence of the  $\text{N}$  of the  $\text{NR}_n\text{N}$  group not satisfied by  $\text{R}$  groups and the  $\text{CH}_2\text{CH}_2$  group being satisfied by monovalent hydrocarbon radicals,

$n$  is an integer from 1 to 2 inclusive and

$\text{X}$  is of the group divalent hydrocarbon radicals and divalent radicals attached to the  $\text{S}$  by a CS linkage, and being composed of C, H and O atoms in the form of ether linkages and

(2) Alkali metal salt of an aliphatic hydrocarbon siliconate having an average of .9 to 1.3 hydrocarbon radicals per silicon atom, said hydrocarbon radicals having from 1 to 4 inclusive carbon atoms, in amount such that the weight pickup of (1) and (2) on the fabric is at least 1% by weight and .5% by weight respectively and thereafter heating the treated fabric to a degree sufficient to give a crease resistant and water repellent fabric.

In carrying out the process of this invention the cellulosic fabric such as cotton, rayon, acetate, linen, or the like or blends of cellulosic fibers with other fibers such as cotton and polyester, is contacted in any desired

2

manner with an aqueous dispersion of (1) and (2). Thus, the fabric can be dipped, sprayed or padded with the dispersion. After the fabric has been saturated with the dispersion, it is then dried and heated to such an extent that the sulfone reacts with the cellulose to crosslink it imparting the crease resistant property. At the same time the siliconate makes the fabric water repellent. In general, it is satisfactory to heat the fabric at temperatures ranging from 100 to 400° F. or higher depending upon the sulfone employed, although temperatures above or below this range are often operative.

In order for the sulfone to operate it is essential that the treating medium be alkaline. When the siliconate is employed in amount of at least 1% by weight of the treating solution, it alone will furnish sufficient alkalinity to cause the sulfone to react with the cellulose. However, when the siliconate is employed in an amount less than 1%, it is often desirable to add additional alkali to the solution in the form of materials such as sodium hydroxide or potassium carbonate in order to obtain the desired degree of alkalinity. If desired, additional alkali can be employed in any event.

For a more detailed description of the alkaline conditions needed for reacting the sulfones with the cellulose, reference may be had to the publications of G. C. Tesoro et al. in the "Textile Research Journal," volume 31, 283 (1961), volume 32, 18 (1962), and volume 33, 93 (1963). These publications also set forth a wide variety of sulfones which can be employed in this invention.

The sulfones which are operative in this invention are divinylsulfone and sulfones of the formula



in which  $\text{Z}$  can be thiosulfate salt groups of the formula  $\text{SSO}_3\text{M}$ , in which  $\text{M}$  can be any anion such as sodium, potassium, ammonium, cesium, or other metals. Preferably the anion is one which will render the sulfone water soluble or at least water dispersible.  $\text{Z}$  can also be the sulfate group  $-\text{OSO}_3\text{M}$  where  $\text{M}$  is any anion as shown above.  $\text{Z}$  can also be any quaternary ammonium salt residue such as those derived from pyridine hydrochloride, quinoline hydrochloride, trimethylamine, ethyldimethylamine, benzylidimethylamine, allyldiethylamine, or any other tertiary amine. Finally,  $\text{Z}$  can be a hydroxyl, a lower alkoxy group such as methoxy, ethoxy, butoxy, or 2-ethylhexoxy or an unsaturated aliphatic hydrocarbonoxy group such as allyloxy or hexenylxy or  $\text{Z}$  can be an acyl group derived from any lower aliphatic carboxylic acid. Examples of such groups are formyl, acetyl, propiophenyl, acrylyl or methacrylyl.

In addition to the above monosulfones, (1) can also be disulfones of the formula



where  $\text{Z}$  is above defined and  $\text{X}$  is any divalent hydrocarbon radical such as methylene, dimethylene, tetramethylene, hexamethylene, octamethylene, or  $\text{CH}_2\text{CH}=\text{CHCH}_2$ ,  $\text{CH}_2\text{CH}_2\text{CH}=\text{CHCH}_2\text{CH}_2$ , phenylene, cyclohexylene, methylcyclohexylene, tolylene, or biphenylene.  $\text{X}$  can also be a hydrocarbon ether radical such as



and



(1) Can also be a disulfone of the formula



in which  $\text{R}$  is a divalent hydrocarbon radical. The  $\text{NR}_n\text{N}$  grouping is derived from a bis-secondary amine and can be of two types. When  $n$  is 1, the group has the formula



in which R is a divalent hydrocarbon radical, and R'' is a monovalent hydrocarbon radical. These groups, of course, are derived from linear bis-secondary amines. The second type of NR<sub>n</sub>N group arises when n is 2. In this case, the group is of a cyclic structure and there are two monovalent hydrocarbon radicals between the nitrogens, the latter, of course, being a part of the cyclic structure. These groups are derived from bis-secondary cyclic amines such as



in which x is an integer. Specific examples of such amines are those in which x is 2, 3 and 5.

Ingredient (2) can be any alkali metal salt of an aliphatic hydrocarbon silicate in which the hydrocarbon groups are from 1 to 4 carbon atoms. This would include siliconates such as methyl silicate, ethyl silicate, vinyl silicate, allyl silicate, propyl silicate, isopropyl silicate, and butyl silicate. If desired, the silicates can contain some unsubstituted silicon atoms and some di-substituted silicon atoms such as dimethylsilicate, ethylmethylsilicate, methylvinyl silicate, etc. Also some of the silicon atoms in the silicate structure can be linked through alkylene bridges in which the bridges are methylene, ethylene, trimethylene, or butylene. The above alkali metal siliconates are well-known materials and are available commercially.

For the purpose of this invention there should be an average of from .9 to 1.3 total hydrocarbon radicals per silicon in the silicate. The alkali metal can be any alkali metal such as lithium, sodium, potassium or cesium and the alkali metal can be present in ratios from 1 to 3 alkali metal atoms per silicon. The solubility of the alkali metal silicate varies with the alkali metal and with the size and number of hydrocarbon groups attached to the silicon. In general, the lithium salts are the least soluble and the cesium salts are most soluble of the alkali metal siliconates. Thus, in those salts where the hydrocarbon group totals 4 carbon atoms, it is preferable to use the potassium or cesium salts rather than the sodium or lithium salts.

For the purpose of this invention the amount of (1) and (2) employed should be such that the fabric will pickup at least 1% by weight of (1) and at least 1/2% by weight of (2). The upper limit of these ingredients is not critical although for cost reasons it is preferable that the fabric contain no more than 5% by weight silicone. In general, (1) should be employed in amount of from 1 to 10% by weight although more can be employed if desired.

Fabrics treated in accordance with this invention are both crease resistant and water repellent and they retain these properties after repeated washings. Consequently, the fabrics so treated are useful in a wide variety of applications.

The following examples are illustrative only and should not be construed as limiting the invention which is properly delineated in the appended claims.

The crease recovery of the fabrics in the following examples was determined in accordance with AATCC Method 66-1959T and the spray rating was determined in accordance with AATCC Method 22-1964.

#### Example 1

A solution of 9.37 g. of bis-beta-hydroxyethyl sulfone and 1.87 g. of sodium methyl silicate diluted to 100 g. in distilled water was prepared. Samples of 80 x 80 cotton cloth were padded with this solution, air dried and cured 1 1/2 minutes at 350° F. The cured samples were bleached with hydrogen peroxide (2%) in a .5%

by weight Tide solution. The bleached fabric was rinsed with warm water and air dried. The spray rating was determined and the crease recovery angles measured after overnight conditioning in a constant temperature room at 72° F. and 50% relative humidity. The crease recovery angle is the sum of the average of three measurements in the warp and three measurements in the fill directions of the fabric. For comparison a run was made in which no alkaline material was added to the bath and one was made in which sodium carbonate was used in place of the silicate.

| 15 | Catalyst                              | Crease Recovery, deg. | Spray Rating |
|----|---------------------------------------|-----------------------|--------------|
|    | None.....                             | 163                   | 0            |
|    | Na <sub>2</sub> CO <sub>3</sub> ..... | 253                   | 80           |
|    | Sodium methyl silicate.....           | 266                   |              |

#### Example 2

The procedure of Example 1 was repeated employing 8% bis-beta-hydroxyethyl sulfone and varying concentrations of sodium methyl silicate and sodium propyl silicate as shown below.

| 30 | Percent Pickup on Fabric    | Crease Recovery, deg. | Spray Rating |
|----|-----------------------------|-----------------------|--------------|
|    | Sodium methyl silicate..... | 1 226                 | 70           |
| 35 | 2 267                       | 80                    |              |
|    | Sodium propyl silicate..... | 1 239                 | 70           |
|    | 2 258                       | 80                    |              |

#### Example 3

The durability of the treatment of this invention is shown in this example. Following the procedure of Example 1, a sample 80 x 80 cotton was padded with a solution of bis-beta-hydroxyethyl sulfone and sodium methyl silicate. The treated fabric was laundered in a Westinghouse Washer at 150° F., with Tide detergent. Spray ratings were determined on the fabric after the initial treatment and after 1, 3 and 5 launderings.

| 50 | Washes       | Crease Recovery, deg. | Spray Rating |
|----|--------------|-----------------------|--------------|
|    | Initial..... | 243                   | 80           |
| 55 | 1.....       | 234                   | 70           |
|    | 3.....       | 255                   | 70           |
|    | 5.....       | 243                   | 70           |

#### Example 4

A solution was made by dissolving 9.37 g. of bis-beta-hydroxyethyl sulfone and 1.87 g. of potassium butyl silicate in 100 g. of distilled water containing some ethanol. 80 x 80 cotton cloth was padded in accordance with the procedure of Example 1. The fabric was then laundered under the conditions of Example 3. The results are as follows:

| 70 | Washes       | Crease Recovery, deg. | Spray Rating |
|----|--------------|-----------------------|--------------|
|    | Initial..... | 253                   | 80           |
|    | 1.....       | 250                   | 70           |
| 75 | 3.....       | 287                   | 50           |

5  
Example 5

Equivalent results are obtained when sodium vinyl silicate and a silicate composed of a mixture of sodium ethyl silicate and one of the structure



are employed in the procedure of Example 1.

## Example 6

A combination of crease resistance and water repellency is obtained when cotton fabric is treated with a mixture of sodium methyl silicate and the following sulfones:



That which is claimed is:

1. The method comprising contacting a cellulosic fabric with an aqueous dispersion of a mixture of
  - (1) a sulfone selected from the group consisting of divinyl sulfone,  $\text{CH}_2=\text{CHSO}_2\text{CH}_2\text{CH}_2\text{Z}$ ,  $\text{ZCH}_2\text{CH}_2\text{SO}_2\text{CH}_2\text{CH}_2\text{Z}$ ,  $\text{ZCH}_2\text{CH}_2\text{SO}_2\text{XSO}_2\text{CH}_2\text{CH}_2\text{Z}$  and  $\text{CH}=\text{CHSO}_2\text{CH}_2\text{CH}_2\text{NR}_n\text{NCH}_2\text{CH}_2\text{SO}_2\text{CH}=\text{CH}_2$  in which  $\text{Z}$  is selected from the group consisting of  $-\text{SSO}_3\text{M}$ ,  $-\text{OSO}_3\text{M}$ , quarternary ammonium salt residues attached to the  $\text{CH}_2\text{CH}_2$  group

## 6

through a carbon-nitrogen bond and  $\text{OR}'$  groups, in which

$\text{M}$  is an anion,

$\text{R}'$  is selected from the group consisting of hydrogen, lower aliphatic hydrocarbon radicals and acyl radicals derived from lower aliphatic carboxylic acids,

$\text{R}$  is a divalent hydrocarbon radical, any valence of the nitrogen of the group  $\text{NR}_n\text{N}$  not satisfied by  $\text{R}$  groups and the  $\text{CH}_2\text{CH}_2$  group being satisfied by monovalent hydrocarbon radicals,

$n$  is an integer from 1 to 2 inclusive, and  $\text{X}$  is selected from the group consisting of divalent hydrocarbon radicals and divalent radicals attached to the  $\text{S}$  by a  $\text{CS}$  linkage and being composed of carbon, hydrogen and oxygen atoms in the form of ether linkages and

(2) an alkali metal salt of an aliphatic hydrocarbon silicate having an average of from .9 to 1.3 hydrocarbon radicals per silicon, said hydrocarbon radicals having from 1 to 4 inclusive carbon atoms in amount such that the weight pickup of (1) and (2) on the fabric is at least 1% by weight and .5% by weight respectively and thereafter heating the treated fabric to a degree sufficient to give a crease resistant and water repellent fabric.

2. The process in accordance with claim 1 in which the sulfone is bis-beta-hydroxyethyl sulfone.

3. The method in accordance with claim 1 in which (1) is bis-beta-hydroxyethyl sulfone and (2) is sodium methyl silicate.

4. The method in accordance with claim 1 in which (1) is bis-beta-hydroxyethyl sulfone and (2) is sodium propyl silicate.

35. 5. As a composition of matter an aqueous dispersion containing at least 1% by weight based on the weight of the dispersion of composition (1) of claim 1 and at least .5% by weight based on the weight of the dispersion of composition (2) of claim 1.

40. 6. The composition in accordance with claim 5 in which (1) is bis-beta-hydroxyethyl sulfone.

7. The composition in accordance with claim 5 in which (1) is bis-beta-hydroxyethyl sulfone and (2) is sodium methyl silicate.

45. 8. The composition in accordance with claim 5 in which (1) is bis beta-hydroxyethyl sulfone and (2) is sodium propyl silicate.

9. A fabric treated in accordance with claim 1.

10. A fabric treated in accordance with claim 2.

11. A fabric treated in accordance with claim 3.

12. A fabric treated in accordance with claim 4.

## References Cited

## UNITED STATES PATENTS

|    |           |         |                 |       |         |
|----|-----------|---------|-----------------|-------|---------|
| 55 | 3,000,762 | 9/1961  | Tesoro          | ----- | 8-120 X |
|    | 3,031,435 | 4/1962  | Tesoro          | ----- | 8-120 X |
|    | 3,178,250 | 4/1965  | Ellis et al.    |       |         |
|    | 3,194,627 | 7/1965  | Gagarine        | ----- | 8-120 X |
| 60 | 3,218,118 | 11/1965 | Steele et al.   | ----- | 8-120 X |
|    | 3,222,119 | 12/1965 | Tashlick et al. | ----- | 8-120 X |

NORMAN G. TORCHIN, Primary Examiner.

J. CANNON, Assistant Examiner.